



US006248507B1

(12) **United States Patent**  
Budz et al.

(10) **Patent No.:** US 6,248,507 B1  
(45) **Date of Patent:** Jun. 19, 2001

(54) **COMPOSITE SILVER HALIDE GRAINS WITH IMPROVED RECIPROCITY AND PROCESS FOR THEIR PREPARATION**

(75) Inventors: **Jerzy A. Budz**, Fairport; **Seshadri Jagannathan**, Pittsford; **Alan R. Sadler**, Hilton, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/475,839**

(22) Filed: **Dec. 30, 1999**

(51) **Int. Cl.<sup>7</sup>** ..... **G03C 1/005**

(52) **U.S. Cl.** ..... **430/363; 430/569; 430/567**

(58) **Field of Search** ..... **430/567, 569, 430/363**

(56) **References Cited**

U.S. PATENT DOCUMENTS

|             |         |                              |
|-------------|---------|------------------------------|
| 4,865,962   | 9/1989  | Hasebe et al. .              |
| 5,252,454   | 10/1993 | Suzumoto et al. .            |
| 5,252,456   | 10/1993 | Ohshima et al. .             |
| 5,547,827   | 8/1996  | Chen et al. .                |
| 5,549,879   | 8/1996  | Chow .                       |
| 5,550,013   | 8/1996  | Chen et al. .                |
| 5,605,789   | 2/1997  | Chen et al. .                |
| 5,726,005   | 3/1998  | Chen et al. .                |
| 5,728,516   | 3/1998  | Edwards et al. .             |
| 5,736,310   | 4/1998  | Chen et al. .                |
| 5,783,372   | 7/1998  | Budz et al. .                |
| 5,792,601   | 8/1998  | Edwards et al. .             |
| 6,030,762 * | 2/2000  | Verrept et al. ..... 438/567 |
| 6,048,683   | 4/2000  | Mehta et al. .               |

\* cited by examiner

*Primary Examiner*—Janet Baxter

*Assistant Examiner*—Amanda C. Walke

(74) *Attorney, Agent, or Firm*—Andrew J. Anderson

(57)

**ABSTRACT**

A process for the preparation of a radiation-sensitive silver halide emulsion comprised of high chloride cubical host grains containing from 0.05 to 3 mole percent iodide, based on total silver, and epitaxially deposited silver bromide, where the iodide is incorporated in the host grains in a controlled, non-uniform distribution forming a core containing at least 50 percent of total silver, an iodide free surface shell having a thickness of greater than 50 Å, and a sub-surface shell that contains a maximum iodide concentration is disclosed, the process comprising: (a) providing in a stirred reaction vessel a dispersing medium and high chloride silver halide cubical grains which form the high chloride host grain cores, (b) adding fine silver iodide grains to the reaction vessel and ripening out the fine silver iodide grains to form the sub-surface shells that contain a maximum iodide concentration, (c) precipitating silver chloride onto the sub-surface shells to form an iodide free surface shell, and (d) depositing silver bromide in an amount of from 0.05 to 5 mole percent, based on total silver, on the host grain surfaces in the presence of an iridium dopant. Also disclosed are photographic recording elements comprising a support and at least one light sensitive silver halide emulsion layer comprising silver halide grains prepared as described above, and an electronic printing method which comprises subjecting a radiation sensitive silver halide emulsion layer of a recording element to actinic radiation of at least  $10^{-4}$  ergs/cm<sup>2</sup> for up to 100μ seconds duration in a pixel-by-pixel mode, wherein the silver halide emulsion layer is comprised of silver halide grains prepared as described above.

**23 Claims, No Drawings**

**COMPOSITE SILVER HALIDE GRAINS  
WITH IMPROVED RECIPROCITY AND  
PROCESS FOR THEIR PREPARATION**

**FIELD OF THE INVENTION**

This invention is directed to radiation sensitive cubical silver iodochloride emulsions having epitaxially deposited silver bromide, and a process for the preparation thereof.

**DEFINITION OF TERMS**

The term "high chloride" in referring to silver halide grains and emulsions indicates that chloride is present in a concentration of greater than 50 mole percent, based on total silver.

In referring to grains and emulsions containing two or more halides, the halides are named in order of ascending concentrations.

The term "cubic grain" is employed to indicate a grain is that bounded by six {100} crystal faces. Typically the comers and edges of the grains show some rounding due to ripening, but no identifiable crystal faces other than the six {100} crystal faces. The six {100} crystal faces form three pairs of parallel {100} crystal faces that are equidistantly spaced.

The term "cubical grain" is employed to indicate grains that are at least in part bounded by {100} crystal faces satisfying the relative orientation and spacing of cubic grains. That is, three pairs of parallel {100} crystal faces are equidistantly spaced. Cubical grains include both cubic grains and grains that have one or more additional identifiable crystal faces. For example, tetradecahedral grains having six {100} and eight {111} crystal faces are a common form of cubical grains.

The term "central portion" in referring to cubical silver halide grains refers to that portion of the grain structure that is first precipitated accounting for up to 98 percent of total precipitated silver required to form the {100} crystal faces of the grains.

The term "dopant" is employed to indicate any material within the rock salt face centered cubic crystal lattice structure of a silver halide grain other than silver ion or halide ion.

The term "dopant band" is employed to indicate the portion of the grain formed during the time that dopant was introduced to the grain during precipitation process.

The term "normalized" molar addition rate hereinafter assigned the symbol  $R_n$  is a measure of the intensity of rate of addition of silver salt solution to the reaction vessel in case of a double-jet precipitation process.  $R_n$  is defined by the formula:

$$R_n = Q_f C_f / M$$

where  $Q_f$  is the volumetric rate (liters/min) of addition of silver salt solution into the reaction vessel,  $C_f$  is the molar concentration (moles/liter) of the said solution, and  $M$  is total moles of silver halide host grains in the reaction vessel at the precise moment of above addition.

All references to the periodic table of elements periods and groups in discussing elements are based on the Periodic Table of Elements as adopted by the American Chemical Society and published in the *Chemical and Engineering News*, Feb. 4, 1985, p. 26. The term "Group VIII" is used to generically describe elements in groups 8, 9 and 10.

The term "log E" is the logarithm of exposure in lux-seconds.

Photographic speed is reported in relative log units and therefore referred to as relative log speed. 1.0 relative log speed unit is equal to 0.01 log E.

The term "contrast" or "γ" is employed to indicate the slope of a line drawn from stated density points on the characteristic curve.

The term "reciprocity law failure" refers to the variation in response of an emulsion to a fixed light exposure due to variation in the specific exposure time.

10 *Research Disclosure* is published by Kenneth Mason Publications, Ltd., Dudley House, 12 North St., Emsworth, Hampshire PO10 7DQ, England.

**BACKGROUND**

15 In its most commonly practiced form silver halide photography employs a film in a camera to produce, following photographic processing, a negative image on a transparent film support. A positive image for viewing is produced by exposing a photographic print element containing one or more silver halide emulsion layers coated on a reflective white support through the negative image in the camera film, followed by photographic processing. In a relatively recent variation negative image information is retrieved by scanning and stored in digital form. The digital image information is later used to expose imagewise the emulsion layer or layers of the photographic print element.

Whereas high bromide silver halide emulsions are the overwhelming commercial choice for camera films, high chloride cubic grain emulsions are the overwhelming commercial choice for photographic print elements. It is desired in high chloride emulsions for color paper applications to obtain high photographic speed at the desired curve shape. While it has been common practice to avoid or minimize the incorporation of iodide into high chloride grains employed

30 in color paper, it has been recently observed that silver iodochloride cubical grains can offer exceptional levels of photographic speed where iodide is incorporated in such emulsion gains in a profiled manner. Chen et. al. in U.S. Pat. No. 5,547,827; Chen et. al. in U.S. Pat. No. 5,550,013; Chen

35 et. al. in U.S. Pat. No. 5,605,789; Chen et. al. in U.S. Pat. No. 5,726,005; Edwards et.al. in U.S. Pat. No. 5,728,516; Chen et. al. in U.S. Pat. No. 5,736,310; Budz et.al. in U.S. Pat. No. 5,783,372 and Edwards et.al. in U.S. Pat. No. 5,792,601 disclose highly sensitive silver iodochloride cubical emulsions with low levels of iodide located in the exterior portions of the grains. The interior portions of such grains can be prepared by employing any convenient high chloride cubic grain precipitation procedure. The emulsion grains thus formed then serve as hosts for further growth. Once a

40 host grain population has been prepared, an increased concentration of iodide is introduced into the emulsion to form the region of the grains containing maximum iodide concentration. The source of iodide ion can be silver iodide grains or any iodide-releasing agent, but it is typically disclosed that iodide is preferably introduced alone as an aqueous solution of an alkali metal iodide salt. This is followed by double-jet introduction of silver nitrate and alkali metal chloride solutions at conventional molar addition rates, constant or ramped, till the exterior portion is 45 grown to the desired size.

Many known imaging systems require that a hard copy be provided from an image which is in digital form. A typical example of such a system is electronic printing of photographic images which involves control of individual pixel exposure. Such a system provides greater flexibility and the opportunity for improved print quality in comparison to optical methods of photographic printing. In a typical elec-

tronic printing method, an original image is first scanned to create a digital representation of the original scene. The data obtained is usually electronically enhanced to achieve desired effects such as increased image sharpness, reduced graininess and color correction. The exposure data is then provided to an electronic printer which reconstructs the data into a photographic print by means of small discrete elements (pixels) that together constitute an image. In a conventional electronic printing method, the recording element is scanned by one or more high energy beams to provide a short duration exposure in a pixel-by-pixel mode using a suitable source such as a cathode ray tube (CRT), light emitting diode (LED) or laser. Such methods are described in the patent literature, including, for example, Hioki U.S. Pat. No. 5,126,235; European Patent Application 479 167 A1 and European Patent Application 502 508 A1. Also, many of the basic principles of electronic printing are provided in Hunt, *The Reproduction of Colour*, Fourth Edition, pages 306-307, (1987).

Reciprocity characteristics, usually referred to as reciprocity failure, are measured in terms of departures from the law of photographic reciprocity. The exposure (E) of a photographic element is the product of the intensity (I) of exposure multiplied by its duration (time):

$$E = I \times t$$

According to the photographic law of reciprocity, a photographic element should produce the same image with the same exposure, even though exposure intensity and time are varied. For example, an exposure for  $\frac{1}{100}$ th of a second at a selected intensity should produce exactly the same result as an exposure of  $10^{-5}$  second at an intensity that is increased by a factor of  $10^3$ . When photographic performance is noted to diverge from the reciprocity law, this is known as reciprocity failure.

A very typical observation in examining high chloride emulsions for photographic print applications is that speed declines at equal exposures as the intensity of exposure increases. For equal exposures, a speed difference at the exposure time of  $10^{-5}$  second or less, as compared to an exposure time of  $\frac{1}{100}$ th of a second is commonly referred to in the art as high intensity reciprocity failure (HIRF). Likewise, the exposure times greater than  $\frac{1}{100}$ th second are often referred to as "long time" exposure, whereas those shorter than that as "short time" exposures.

In order to increase the output of digital printing devices, such as CRT, LED, or laser-based printers it is highly desirable to increase speed of high chloride silver halide emulsions when exposed at very short times even further. In the art of silver chloride-based color paper preparation it is the blue color record that has the greatest need for speed.

The use of dopants in silver halide grains to modify photographic performance is generally illustrated by *Research Disclosure*, Item 38957, cited above, I. Emulsion grains and their preparation, D. Grain modifying conditions and adjustments, paragraphs (3)-(5). Photographic performance attributes known to be affected by dopants include sensitivity, reciprocity failure, and contrast.

Using empirical techniques the art has over the years identified many dopants capable of increasing photographic speed. Keevert et al U.S. Pat. No. 4,945,035, e.g., was the first to teach the incorporation of a hexacoordination complex containing a transition metal and cyano ligands as a dopant in high chloride grains to provide increased sensitivity. Careful scientific investigations have revealed Group VIII hexahalo coordination complexes to create electron traps, as illustrated R. S. Eachus, R. E. Graves and M. T.

Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). Doping with iridium hexachloride complexes, e.g., is commonly performed to reduce reciprocity law failure in silver halide emulsions. The use of iridium dopants containing at least one organic ligand has also been proposed. Specific iridium dopants include those illustrated in high chloride emulsions by Bell U.S. Pat. Nos. 5,474,888, 5,470,771 and 5,500,335 and McIntyre et al U.S. Pat. No. 5,597,686; those disclosed in Olm et al U.S. Pat. Nos. 5,360,712 and 5,457,021; Kuromoto et al U.S. Pat. No. 5,462,849; Mydlarz et al U.S. Pat. No. 5,783,373 and U.S. Pat. No. 5,783,378; Hahm et al U.S. Pat. No. 5,962,210. Specific combinations of iridium and other metal dopants may additionally be found in U.S. Pat. Nos. 4,828,962, 5,153,110, 5,219,722, 5,227,286, and 5,229,263, copending, commonly assigned U.S. Ser. No. 09/250,200 of Mydlarz et al., filed Feb. 16, 1999, and European Patent Applications EP 0 244 184, EP 0 405 938, EP 0 476 602, EP 0 488 601, EP 0 488 737, EP 0 513 748, and EP 0 514 675.

In general, the prior art dopant teachings typically use silver chloride as a host medium and merely disclose that photographic emulsions may contain a variety of halides, including silver iodochloride. They do not, in general, even reference silver iodochloride emulsions in accordance with this invention (those with local regions of high iodide concentration resulting from the rapid addition of iodide ion at some point during the second half of grain formation).

To further improve the photographic performance of high chloride emulsions bromide is often introduced during the process of chemical sensitization or ripening. Hasebe et al U.S. Pat. No. 4,865,962 (a) provides regular grains that are at least 50 (preferably at least 90) mole percent chloride, (b) adsorbs an organic compound to the grain surfaces and (c) introduces bromide, thereby achieving halide conversion (bromide ion displacement of chloride) at selected grain surface sites. Asami EPO 0 295439 discloses the addition of bromide to achieve halide conversion at the surface of silver bromochloride grains that have, prior to halide conversion, a layered structure with the surface portions of the grains having a high chloride concentration. The grains are preferably monodisperse. Suzumoto et al U.S. Pat. No. 5,252,454 discloses silver bromochloride emulsions in which the chloride content is 95 (preferably 97) mole percent or more. The grains contain a localized phase having a bromide concentration of at least 20 mole percent preferably formed epitaxially at the surface of the grains. The grains are preferably monodisperse. Oshima et al U.S. Pat. No. 5,252,456 discloses silver bromochloride emulsions in which the chloride content is at least 80 (preferably equal or greater than 95) mole percent chloride, with a bromide rich phase containing at least 10 mole percent bromide formed at the surface of the grains by blending a fine grain emulsion with a larger host (preferably cubic or tetradecahedral) grain emulsion and Ostwald ripening. An iridium coordination complex containing at least two cyano ligands is employed to increase speed and reduce reciprocity failure.

Edwards et al U.S. Pat. No. 5,792,601 discloses a radiation sensitive emulsion containing iridium doped composite silver halide grains comprised of (a) host portions having an average aspect ratio of less than 1.3 and consisting essentially of monodisperse silver iodochloride grains containing from 0.05 to 3 mole percent iodide, based on total silver forming the host portions, with maximum iodide concentrations located nearer the surface of the host portions than their center and (b) epitaxially deposited portions containing an

iridium dopant and silver bromide accounting for from 0.1 to 5 mole percent of total silver forming the composite grain. The source of iodide used to prepare the host iodochloride portions in all the inventive examples is potassium iodide solution.

It has become increasing clear that with the continuing development of a variety of high intensity digital printing devices that photographic print materials with performance invariant to exposure time is increasingly important. When exposure times are reduced below one second to very short intervals (e.g.,  $10^{-5}$  second or less), higher exposure intensities must be employed to compensate for the reduced exposure times. High intensity reciprocity failure (hereinafter also referred to as HIRF) occurs when photographic performance is noted to depart from the reciprocity law when such shorter exposure times are employed. Print materials which traditionally suffer speed or contrast losses at short exposure times (high intensity exposures) will fail to reproduce detail with high resolution. Text will appear blurred. Through-put of digital print devices will suffer as well. Accordingly, print materials with reduced HIRF are desired in order to produce excellent photographic prints in a wide variety of digital printers.

In addition to reducing HIRF, it is also desirable to reduce low intensity reciprocity failure (LIRF) in photographic elements. Print materials with reduced LIRF, e.g., will allow enlargements of photographs to be made by conventional optical printing techniques with a more faithful matching of image tone and color.

#### PROBLEM TO BE SOLVED BY THE INVENTION

Accordingly, a current challenge in the manufacture of photographic materials, and in particular color photographic print materials such as photographic color paper, is to develop silver iodochloride emulsions with enhanced photographic sensitivity while controlling the reciprocity characteristics. The enhanced sensitivity emulsions are useful to build specific photographic elements that would perform equally well at long time and short time flash exposures of traditional color print materials, as well as extremely short time pixel-by-pixel exposures of digital printing devices. However, while increasing emulsion photographic sensitivity difficulties in maintaining reciprocity are often encountered.

The objective of the present invention is to provide silver halide emulsions comprising cubical silver iodochloride host grains with epitaxially deposited silver bromide with enhanced sensitivity and reciprocity characteristics.

A further objective is to provide color papers that have improved photographic response regardless of the image-wise exposure they have received.

A still further objective is to improve the efficiency of the method of electronic printing using pixel-by-pixel digital short time exposures.

#### SUMMARY OF THE INVENTION

In one aspect this invention is directed towards a process for the preparation of a radiation-sensitive silver halide emulsion comprised of high chloride cubical host grains containing from 0.05 to 3 mole percent iodide, based on total silver, and epitaxially deposited silver bromide, where the iodide is incorporated in the host grains in a controlled, non-uniform distribution forming a core containing at least 50 percent of total silver, an iodide free surface shell having a thickness of greater than 50 Å, and a sub-surface shell that contains a maximum iodide concentration, the process comprising:

- (a) providing in a stirred reaction vessel a dispersing medium and high chloride silver halide cubical grains which form the high chloride host grain cores,
- (b) adding fine silver iodide grains to the reaction vessel and ripening out the fine silver iodide grains to form the sub-surface shells that contain a maximum iodide concentration,
- (c) precipitating silver chloride onto the sub-surface shells to form an iodide free surface shell, and
- (d) depositing silver bromide in an amount of from 0.05 to 5 mole percent, based on total silver, on the host grain surfaces in the presence of an iridium dopant.

In a second aspect, this invention is directed towards a photographic recording element comprising a support and at least one light sensitive silver halide emulsion layer comprising silver halide grains prepared as described above.

In another aspect, this invention is directed to an electronic printing method which comprises subjecting a radiation sensitive silver halide emulsion layer of a recording element to actinic radiation of at least  $10^{-4}$  ergs/cm<sup>2</sup> for up to 100 $\mu$  seconds duration in a pixel-by-pixel mode, wherein the silver halide emulsion layer is comprised of silver halide grains prepared as described above.

The advantages of the invention are generally accomplished by the new method of the preparation of cubical iodochloride grains in combination with epitaxial deposition of silver bromide and iridium dopant. We have discovered that speed and reciprocity of these emulsions can be improved when the source of iodide used for formation of the high iodide concentration region of the iodochloride grains is fine silver iodide grains instead of commonly used potassium iodide solutions.

In a preferred practical application, the advantages of the invention can be transformed into increased throughput of digital artifact-free color print images while exposing each pixel sequentially in synchronism with the digital data from an image processor.

#### DESCRIPTION OF PREFERRED EMBODIMENTS

The cubical silver halide grains precipitated in accordance with the invention contain greater than 50 mole percent chloride, based on silver.

Preferably the grains contain at least 70 mole percent chloride and, optimally at least 90 mole percent chloride, based on silver. Overall iodide concentration is from 0.05 to 3 mole percent, preferably 0.1 to 1 mole percent, based on silver. Silver bromide and silver chloride are miscible in all proportions. Hence, any portion of the total halide not accounted for chloride and iodide, can be bromide. The cubical grains have silver bromide in the amount of from 0.05 to 5 mole percent, based on total silver, more preferably from 0.1 to 1 mole percent, deposited thereon, wherein the silver bromide is deposited in the presence of an iridium dopant. For color reflection print (i.e., color paper) uses bromide is typically limited to less than 10 mole percent based on silver and iodide is preferably limited to less than 1 mole percent based on silver.

It has been recognized for the first time that heretofore unattained levels of sensitivity and other advantageous properties, such as those recited in the objects and demonstrated in the samples below, can be realized, without offsetting degradation of photographic performance, when the source of iodide used for formation of a high iodide concentration region in the iodochloride grains is fine silver iodide grains instead of commonly used potassium iodide

solutions and silver bromide is epitaxially deposited on the surface of the iodochloride grains in the presence of iridium dopant.

In accordance with the emulsions of the invention, iodide addition onto core portions of the grains creates a silver iodochloride shell on the host (core) high chloride grains. Attempts to use these shelled grains in photographic print elements without further modification results in markedly inferior performance. Having high iodide concentrations at the surface of the grains lowers speed as compared to the emulsions satisfying the requirements of the invention when both emulsions are sensitized to the same minimum density and otherwise produces elevated levels of minimum density that are incompatible with acceptable performance characteristics of photographic reflective print elements.

To increase speed and lower minimum density an iodide-free shell is precipitated onto the silver iodochloride shell, converting it into a sub-surface shell. The depth to which sub-surface shell is buried is chosen to render the iodide in the sub-surface shell inaccessible to the developing agent at the outset of development of latent image bearing grains and inaccessible throughout development in the grains that do not contain a latent image. The thickness of the surface shell is contemplated to be greater than 50 Å in emulsions employed in reflection print photographic elements. The surface shell thickness can, of course, range up to any level compatible with the minimum core requirement of 50 (preferably 85) percent of total silver. Since the sub-surface shell can contribute as little as 0.05 mole percent iodide, based on total silver, it is apparent that surface shells can account for only slightly less than all of the silver not provided by the core portions of the grains. A surface shell accounting for just less than 50 (preferably just less than 15) percent of total silver is specifically contemplated. Whereas it might be thought that shifting the maximum iodide phase to the interior of the grain would also shift the latent image internally, detailed investigations have revealed that latent image formation remains at the surface of the grains.

It was initially observed that, after starting with monodisperse silver chloride cubic grains (i.e., grains consisting of six {100} crystal faces), iodide introduction produced tetradecahedral grains (i.e., grains consisting of six {100} crystal faces and eight {111} crystal faces). Further investigations revealed that as few as one {111} crystal face are sometimes present in the completed grains. On still further investigation, it has been observed that the emulsions of the invention can be cubic grain emulsions. Thus, although the presence of at least {111} crystal face (and usually tetradecahedral grains), provides a convenient visual clue that the grains may have been prepared according to the teaching of this invention, it has now been concluded that one or more {111} crystal faces are a by-product of grain formation that can be eliminated or absent without compromising the unexpected performance advantages of the invention noted above.

The preparation of cubical grain silver iodochloride emulsions with iodide placements that produce increased photographic sensitivity can be undertaken by employing any convenient conventional high chloride cubical grain precipitation procedure prior to precipitating the region of maximum iodide concentration—that is, through the introduction of at least the first 50 (preferably at least the first 85) percent of silver precipitation. The initially formed high chloride cubical grains then serve as hosts for further grain growth. In one specifically contemplated preferred form the host emulsion is a monodisperse silver chloride cubic grain emulsion. Low levels of iodide and/or bromide, consistent

with the overall composition requirements of the grains, can also be tolerated within the host grains. The host grains can include other cubical forms, such as tetradecahedral forms. Techniques for forming emulsions satisfying the host grain requirements of the preparation process are well known in the art. For example, prior to growth of the maximum iodide concentration region of the grains, the precipitation procedures of Atwell U.S. Pat. No. 4,269,927, Tanaka EPO 0 080 905, Hasebe et al U.S. Pat. No. 4,865,962, Asami EPO 0 295 439, Suzumoto et al U.S. Pat. No. 5,252,454 or Ohshima et al U.S. Pat. No. 5,252,456, the disclosures of which are here incorporated by reference, can be employed, but with those portions of the preparation procedures, when present, that place bromide ion at or near the surface of the grains being omitted. Stated another way, the host grains can be prepared employing the precipitation procedures taught by the citations above through the precipitation of the highest chloride concentration regions of the grains they prepare. The rate at which silver nitrate and sodium chloride are added into the reactor can be at any practical "normalized" molar addition rate range, including low (R<sub>n</sub> less than or equal to 0.03 min<sup>-1</sup>) and high (R<sub>n</sub> greater than 0.03 min<sup>-1</sup>) addition rates.

Once a host grain population has been prepared accounting for at least 50 percent (preferably at least 85 percent) of total silver has been precipitated, an increased concentration of iodide is introduced into the emulsion to form the region of the grains containing a maximum iodide concentration. In accordance with the invention, the iodide ions are introduced during emulsion preparation by the addition of relatively fine silver iodide seed grains (having a mean grain diameter less than that of the core host grains) which are subsequently ripened out, such as described in *Research Disclosure*, Vol. 531, May 1998, item 40928. To facilitate Ostwald ripening it is contemplated to employ fine grain silver iodide emulsions having a mean grain size of less than 0.1 micrometer. The small sizes of the silver iodide grains are chosen to maximize available grain surface area per unit volume and to improve the distribution of the silver iodide at the time emulsions are blended. In a preferred form the silver iodide grain emulsion is a Lippmann emulsion. Lippmann emulsions with mean grain sizes down to about 30 angstroms have been reported, although the typical mean grain size of Lippmann emulsions is about 0.05 micrometer. While the iodochloride prior art referenced above typically states that any iodide ion source may be used in the preparation thereof, it is a critical feature of the invention that fine silver iodide grains be used as the iodide source for the preparation of the region of the grains containing a maximum iodide concentration.

While not bound to any particular theory, the criticality of the iodide ion source in the process of the invention may be explained as follows. In a conventional process, the first step of the iodide incorporation process is the addition of an aqueous solution of KI. This process results in the formation of a mixture AgI particles (by *in situ* nucleation) and AgClI composite particles (by metathesis). Since the addition of KI solution to the reactor results in a high supersaturation in the reactor, formation of AgI particles predominates over the metathesis reaction during this stage of the process. These AgI particles may exist independently in the emulsion or may be attached as nodules to the AgClI particles. During the subsequent "hold" period after KI addition, the metathesis reaction is dominant, the extent of formation of the AgClI composite particles being determined by the "hold time" and the pCl of the reactor (extent of metathesis being greater at lower pCl values). The supersaturation for the metathesis reaction is inversely related to the pCl of the reactor.

However, the AgI particles formed during the hold period do not completely metathesize during the hold period, when the iodide concentration is greater than 0.05% of the total silver. When silver nitrate and alkali chloride are subsequently added to the reactor, the AgI particles dissolve and coprecipitate on the AgCl(I) substrate particles. Once again, the supersaturation for the coprecipitation process is inversely related to pCl; i.e., it is greater at lower pCl values. In general, precipitation processes may be regulated and controlled better under low supersaturation conditions, while high supersaturation processes can result in an uncontrolled distribution of product species. Since the formation of AgJ particle by the addition of a KI solution to the reactor is a high supersaturation process, this is not a desirable process. In accordance with the invention, the use pre-made AgI particles as the source of iodide provides a low supersaturation alternative and completely avoids (eliminates) the high supersaturation in situ nucleation step. The supersaturation during the subsequent steps in the iodide incorporation process may be minimized by maintaining a high pCl condition and/or adding silver nitrate and alkali chloride at a high addition rate.

The consequence of carrying out the iodide incorporation process under lower supersaturation conditions as described herein is that the generation of uncontrolled and undesirable side products is minimized. As a result, it is possible to increase the concentration of iodide incorporated in the emulsion and achieve improved photographic performance.

To maximize the localization of crystal lattice variances produced by iodide incorporation it is preferred that the iodide ion be introduced as rapidly as possible. That is, the iodide ion forming the maximum iodide concentration region of the grains is preferably introduced in less than 30 seconds, optimally in less than 10 seconds. When the iodide is introduced more slowly, somewhat higher amounts of iodide (but still within the ranges set out above) are required to achieve speed increases equal to those obtained by more rapid iodide introduction and minimum density levels are somewhat higher. Slower iodide additions are manipulatively simpler to accomplish, particularly in larger batch size emulsion preparations. Hence, adding iodide over a period of at least 1 minute (preferably at least 2 minutes) and, preferably, during the concurrent introduction of silver is specifically contemplated.

The rate at which silver salt and halide salt solutions are added to create an outer shell after iodide addition can be at any practical "normalized" molar addition rate range, including low ( $R_n$  less than or equal to  $0.03 \text{ min}^{-1}$ ) and high ( $R_n$  greater than  $0.03 \text{ min}^{-1}$ ) addition rates. Where the reaction vessel contains excess halide ions, the silver salt solution may be added by itself to precipitate the outer shell. It is preferred, however, to simultaneously introduce a halide salt solution into the dispersing medium with the silver salt solution. High normalized molar silver addition rates after iodide addition is the subject of copending, concurrently filed U.S. Ser. No. 09/475,405 (Kodak Docket 80210AJA) of Mehta et al., the disclosure of which is incorporated by reference herein. It is surprising that burying the maximum iodide phase within the grains using high rates of reagents addition not only is compatible with achieving higher levels of photoefficiency but actually contributes an additional increment of speed enhancement.

At the conclusion of grain precipitation the grains can take varied cubical forms, ranging from cubic grains (bounded entirely by six {100} crystal faces), grains having an occasional identifiable {111} face in addition to six {100} crystal faces, and, at the opposite extreme tetradecahedral grains having six {100} and eight {111} crystal faces.

After examining the performance of emulsions exhibiting varied cubical grain shapes, it has been concluded that the performance of these emulsions is principally determined by iodide incorporation and the uniformity of grain size dispersity. The silver iodochloride grains are relatively monodisperse. The silver iodochloride grains preferably exhibit a grain size coefficient of variation of less than 35 percent and optimally less than 25 percent. Much lower grain size coefficients of variation can be realized, but progressively 10 smaller incremental advantages are realized as dispersity is minimized.

Once high chloride cubical grains having profiled iodide concentration have been precipitated as described above, silver bromide is epitaxially deposited thereon in the presence of an iridium dopant. The incorporation of iridium and, optionally, other dopants, after formation of the host grains is achieved by introducing a relatively fine grain emulsion (one having a mean grain diameter less than that of the silver iodochloride grains) containing silver bromide into the host grain emulsion under conditions that allow Ostwald ripening of the fine grains onto the silver iodochloride host grains. To facilitate Ostwald ripening it is contemplated to employ fine grain emulsions having a mean grain size of less than 0.1 micrometer. The small sizes of the silver bromide containing grains are chosen to maximize available grain surface area per unit volume and to improve the distribution of the silver bromide at the time emulsions are blended.

In a preferred form the silver bromide containing emulsion is a Lippmann emulsion. Lippmann emulsions with 30 mean grain sizes down to about 30 angstroms have been reported, although the typical mean grain size of Lippmann emulsions is about 0.05 micrometer.

Silver bromide can be the sole silver halide component of the grains added for Ostwald ripening onto the silver iodochloride host grains. This minimizes the amount of silver halide that must be Ostwald ripened onto the host grains to achieve the required overall bromide concentrations in the composite grains. Except for increasing the total amount of total silver that must be deposited by Ostwald ripening, the inclusion of silver chloride in the fine grains is not objectionable. High (greater than or equal to 50 mole %) bromide emulsions are preferred. Small amounts of iodide, up to about 1 mole percent, based on total silver in the fine grain emulsion, can be tolerated, but it is preferred that the iodide content of the composite grain emulsions be provided entirely by the host grain emulsion.

It is specifically contemplated to dope the fine grain emulsion with iridium and, optionally other dopants, during its precipitation. This simplifies composite grain preparation, since both iridium and silver bromide can be added to the host grain emulsion in a single addition step. If the iridium is not contained in the bromide containing fine grains, it is added to the host grain emulsion no later than the bromide containing fine grains—that is, prior to or concurrently with addition of the fine grains. The use of such doped fine grains is described, e.g., in U.S. Pat. No. 5,792,601 referenced above, the entire disclosure of which is incorporated by reference herein.

Since unnecessarily increasing the bromide concentration of the composite grains diminishes advantages associated with high chloride emulsions, it is preferred to limit the concentrations of silver bromide used to achieve incorporation of the iridium. From the very low levels of iridium required to achieve advantages in accordance with the invention, it is apparent that only very small amounts of bromide ion need be incorporated in the composite grains. It

is generally preferred that the concentration of bromide in the composite grains be in the range of from 0.1 to 1 mole percent, based on the total silver in the composite grains. For the purpose of providing a clear demarcation between the host grain portion and epitaxially deposited silver halide in emulsion grain in accordance with the invention, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

In accordance with the invention, iridium dopants are added to the emulsion grains during chemical sensitization either prior to or with silver bromide epitaxial deposition. The iridium dopant can be introduced in any conventional form and amount known to reduce HIRF. Iridium is preferably introduced as a hexacoordination complex. Generally, where only HIRF improvements are sought by iridium introduction, it is most convenient to introduce iridium as a hexahalocoordination complex. Other ligands are known for iridium dopants, however, and it is in general contemplated to employ as the iridium dopant a hexacoordination complex satisfying the formula:



wherein n is zero, -1, -2, -3 or -4; and  $\text{L}_6$  represents six bridging ligands which can be independently selected, provided that at least four of the ligands are anionic ligands. A net negative charge of the coordination complex is preferred to facilitate its inclusion in the crystal lattice structure. In addition to halide (fluoride, chloride, bromide and/or iodide) ligands, pseudo-halide (e.g., cyano, cyanate, thiocyanate, and/or selenocyanate) ligands can be employed. Subject to anionic ligand requirements, it is also possible to employ various charge neutral ligands, such as aquo and carbonyl ligands. In a specifically preferred form at least four of the ligands are halide ligands, especially chloride or bromide ligands. Additional useful neutral and anionic organic ligands for dopant hexacoordination complexes are also disclosed by Olm et al U.S. Pat. No. 5,360,712 and Kuromoto et al U.S. Pat. No. 5,462,849, the disclosures of which are here incorporated by reference.

When the iridium coordination complex dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated.

The preferred iridium complex for addition during fin- ishing is an iridium hexachloride compound, which is preferably added in an amount between 0.0001 and 1.0 mg/silver mole, more preferably between 0.001 and 0.1 mg/silver mole, for best photographic performance.

While addition of iridium during chemical sensitization is the only dopant addition required for the practice of the invention, it is specifically contemplated to incorporate additional dopants into the silver halide emulsion grains of the invention during precipitation. The use of dopants in

silver halide grains to modify photographic performance is generally illustrated by *Research Disclosure*, Item 38957, cited above, I. Emulsion grains and their preparation, D. Grain modifying conditions and adjustments, paragraphs (3)-(5). Photographic performance attributes known to be affected by dopants include sensitivity, reciprocity failure, and contrast.

In accordance with preferred embodiments of the invention, iridium coordination complex dopants may also be incorporated into the face centered cubic crystal lattice of the host emulsion grains prior to epitaxial deposition of silver bromide. In such instance, the iridium dopant preferably contains at least one thiazole or substituted thiazole ligand. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. In a specifically preferred form the remaining non-thiazole or non-substituted-thiazole ligands of the iridium coordination complex dopants incorporated into the host grains are halide ligands. The iridium dopants are effective at some level at any location within the grains. Generally better results are obtained, however, when the dopant is incorporated in the exterior 50 percent of the grain, based on silver. To insure that the dopant is in fact incorporated in the grain structure and not merely associated with the surface of the grain, it is possible to introduce the dopant prior to forming, during or after forming the maximum iodide concentration region of the grain. In accordance with a preferred embodiment, however, an iridium dopant may be introduced prior to formation of the high iodide band (within a region adjacent to the high iodide band and comprising up to 60% of the total silver into the emulsion grains, preferably up to 40% of the total silver, and most preferably up to 20% of the total silver), or incorporated into the high iodide band by introducing the dopant into the reaction vessel as a single-jet with iodide solution, as disclosed in concurrently filed, copending, commonly assigned U.S. Ser. No. 09/475, 405 (Kodak Docket No. 80209AJA), the disclosure of which is incorporated by reference herein. Generally better results are obtained when the dopant is incorporated in the exterior 50 percent of the grain, based on silver. Thus, an optimum grain region for dopant incorporation is that formed by silver ranging from 0 to 50 percent of total silver prior to iodide addition. That is, dopant introduction is optimally commenced after 50 percent minus the shell volume over iodide band of total silver has been introduced. The dopant can be introduced all at once or run into the reaction vessel over a period of time while grain precipitation is continuing. It is preferred to run dopant over a period of time, thus forming a dopant band within the grain. The iridium dopants incorporated in the host grains can be employed in any conventional useful concentration, and are generally used in an amount between  $1 \times 10^{-10}$  and  $1 \times 10^{-5}$  moles per silver mole. A preferred amount of the iridium is between  $1 \times 10^{-9}$  and  $1 \times 10^{-6}$  moles per silver mole for best photographic performance.

The contrast of photographic elements containing silver iodochloride emulsions of the invention can be further increased by doping the silver iodochloride grains with a hexacoordination complex containing a nitrosyl or thionitrosyl ligand. Preferred coordination complexes of this type are represented by the formula:



where

- T is a Os or Ru;
- E is a bridging ligand;
- E' is E or NZ;
- r is zero, -1, -2 or -3; and
- Z is oxygen or sulfur.

The E ligands can take any of the forms found in the dopants. A listing of suitable coordination complexes satisfying the above formula is found in McDugle et al U.S. Pat. No. 4,933,272, the disclosure of which is here incorporated by reference.

Osmium and ruthenium dopants such as described in U.S. Pat. No. 5,830,631, the disclosure of which is hereby incorporated by reference, may also be used in the emulsions of the invention.

The emulsions can be prepared in any mean grain size known to be useful in photographic print elements. Mean grain sizes in the range of from 0.15 to 2.5  $\mu\text{m}$  are typical, with mean grain sizes in the range of from 0.2 to 2.0  $\mu\text{m}$  being generally preferred.

High chloride cubical grains having profiled iodide concentration and epitaxially deposited silver bromide in accordance with the invention may be further modified by conventional chemical and spectral sensitization, followed by the addition of conventional addenda to adapt the emulsion for the imaging application of choice can take any convenient conventional form. These conventional features are illustrated by *Research Disclosure*, Item 38957, cited above, particularly:

- III. Emulsion washing;
- IV. Chemical sensitization;
- V. Spectral sensitization and desensitization;
- VII. Antifoggants and stabilizers;
- VIII. Absorbing and scattering materials;
- IX. Coating and physical property modifying addenda; and
- X. Dye image formers and modifiers.

The emulsions of the invention may be chemically sensitized as known in the art. Preferred chemical sensitizers include gold and sulfur chemical sensitizers. Typical of suitable gold and sulfur sensitizers are those set forth in Section IV of *Research Disclosure* 38957, September 1996. Preferred is colloid aurous sulfide such as disclosed in *Research Disclosure* 37154 for good speed and low fog.

The emulsions can be spectrally sensitized in any convenient conventional manner. Spectral sensitization and the selection of spectral sensitizing dyes is disclosed, for example, in *Research Disclosure*, Item 38957, cited above, Section V. Spectral sensitization and desensitization. The emulsions used in the invention can be spectrally sensitized with dyes from a variety of classes, including the polymethine dye class, which includes the cyanines, merocyanines, complex cyanines and merocyanines (i.e., tri-, tetra- and polynuclear cyanines and merocyanines), styryls, merostyryls, streptocyanines, hemicyanines, arylidines, allopolar cyanines and enamine cyanines. Combinations of spectral sensitizing dyes can be used which result in supersensitization—that is, spectral sensitization greater in some spectral region than that from any concentration of one of the dyes alone or that which would result from the additive effect of the dyes. Supersensitization can be achieved with selected combinations of spectral sensitizing dyes and other addenda such as stabilizers and antifoggants, development accelerators or inhibitors, coating aids, brighteners and antistatic agents. Any one of several mechanisms,

as well as compounds which can be responsible for supersensitization, are discussed by Gilman, *Photographic Science and Engineering*, Vol. 18, 1974, pp. 418-430.

The silver iodochloride emulsions are preferably protected against changes in fog upon aging. Preferred antifoggants can be selected from among the following groups:

- A. A mercapto heterocyclic nitrogen compound containing a mercapto group bonded to a carbon atom which is linked to an adjacent nitrogen atom in a heterocyclic ring system,
- B. A quaternary aromatic chalcogenazolium salt wherein the chalcogen is sulfur, selenium or tellurium,
- C. A triazole or tetrazole containing an ionizable hydrogen bonded to a nitrogen atom in a heterocyclic ring system, or
- D. A dichalcogenide compound comprising an —X—X— linkage between carbon atoms wherein each X is a divalent sulfur, selenium or tellurium.

The above groups of antifoggants are known in the art, and are described in more detail, e.g., in U.S. Pat. No. 5,792,601, the disclosure of which is incorporated by reference herein.

In the simplest contemplated form a recording element in accordance with the invention can consist of a single emulsion layer satisfying the emulsion description provided above coated on a conventional photographic support, such as those described in *Research Disclosure*, Item 38957, cited above, XVI. Supports. In one preferred form the support is a white reflective support, such as photographic paper support or a film support that contains or bears a coating of a reflective pigment. To permit a print image to be viewed using an illuminant placed behind the support, it is preferred to employ a white translucent support, such as a Duratrans<sup>TM</sup> or Duraclear<sup>TM</sup> support.

The invention can be used to form either silver or dye images in the recording element. In a simple form a single radiation sensitive emulsion layer unit is coated on the support. The emulsion layer unit can contain one or more high chloride silver halide emulsions satisfying the requirements of the invention, either blended or located in separate layers. When a dye imaging forming compound, such as a dye-forming coupler, is present in the layer unit, it can be present in an emulsion layer or in a layer coated in contact with the emulsion layer. With a single emulsion layer unit a monochromatic image is obtained.

It is, of course, recognized that the photographic elements of the invention can include more than one emulsion. Where more than one emulsion is employed, such as in a photographic element containing a blended emulsion layer or separate emulsion layer units, all of the emulsions can be silver iodochloride emulsions as contemplated by this invention. Alternatively one or more conventional emulsions can be employed in combination with the silver iodochloride emulsions of this invention. For example, a separate emulsion, such as a silver chloride or bromochloride emulsion, can be blended with a silver iodochloride emulsion according to the invention to satisfy specific imaging requirements. For example, emulsions of differing speed are conventionally blended to attain specific aim photographic characteristics. Instead of blending emulsions, the same effect can usually be obtained by coating the emulsions that might be blended in separate layers. It is well known in the art that increased photographic speed can be realized when faster and slower emulsions are coated in separate layers with the faster emulsion layer positioned to receiving exposing radiation first. When the slower emulsion layer is coated to receive exposing radiation first, the result is a higher contrast image. Specific illustrations are provided by

*Research Disclosure*, Item 36544, cited above Section I. Emulsion grains and their preparation, Subsection E. Blends, layers and performance categories.

The emulsion layers as well as optional additional layers, such as overcoats and interlayers, contain processing solution permeable vehicles and vehicle modifying addenda. Typically these layer or layers contain a hydrophilic colloid, such as gelatin or a gelatin derivative, modified by the addition of a hardener. Illustrations of these types of materials are contained in *Research Disclosure*, Item 36544, previously cited, Section II. Vehicles, vehicle extenders, vehicle-like addenda and vehicle related addenda. The overcoat and other layers of the photographic element can usefully include an ultraviolet absorber, as illustrated by *Research Disclosure*, Item 36544, Section VI. UV dyes/ optical brighteners/luminescent dyes, paragraph (1). The overcoat, when present can usefully contain matting agents to reduce surface adhesion. Surfactants are commonly added to the coated layers to facilitate coating. Plasticizers and lubricants are commonly added to facilitate the physical handling properties of the photographic elements. Antistatic agents are commonly added to reduce electrostatic discharge. Illustrations of surfactants, plasticizers, lubricants and matting agents are contained in *Research Disclosure*, Item 36544, previously cited, Section IX. Coating physical property modifying addenda.

Preferably the photographic elements of the invention include a conventional processing solution decolorizable antihalation layer, either coated between the emulsion layer (s) and the support or on the back side of the support. Such layers are illustrated by *Research Disclosure*, Item 36544, cited above, Section VIII. Absorbing and Scattering Materials, Subsection B, Absorbing materials and Subsection C. Discharge.

A specific preferred application of the invention is in color photographic elements, particularly color print (e.g., color paper) photographic elements intended to form multicolor images. In multicolor image forming photographic elements at least three superimposed emulsion layer units are coated on the support to separately record blue, green and red exposing radiation. The blue recording emulsion layer unit is typically constructed to provide a yellow dye image on processing, the green recording emulsion layer unit is typically constructed to provide a magenta dye image on processing, and the red recording emulsion layer unit is typically constructed to provide a cyan dye image on processing. Each emulsion layer unit can contain one, two, three or more separate emulsion layers sensitized to the same one of the blue, green and red regions of the spectrum. When more than one emulsion layer is present in the same emulsion layer unit, the emulsion layers typically differ in speed. Typically interlayers containing oxidized developing agent scavengers, such as ballasted hydroquinones or aminophenols, are interposed between the emulsion layer units to avoid color contamination. Ultraviolet absorbers are also commonly coated over the emulsion layer units or in the interlayers. Any convenient conventional sequence of emulsion layer units can be employed, with the following being the most typical:

---

Surface Overcoat  
Ultraviolet Absorber  
Red Recording Cyan Dye Image Forming Emulsion Layer Unit  
Scavenger Interlayer  
Ultraviolet Absorber

-continued

---

|    |                                                               |
|----|---------------------------------------------------------------|
| 5  | Green Recording Magenta Dye Image Forming Emulsion Layer Unit |
| 10 | Scavenger Interlayer                                          |
| 15 | Blue Recording Yellow Dye Image Forming Emulsion Layer Unit   |
| 20 | Reflective Support                                            |

---

10 Further illustrations of this and other layers and layer arrangements in multicolor photographic elements are provided in *Research Disclosure*, Item 36544, cited above, Section XI. Layers and layer arrangements.

15 Each emulsion layer unit of the multicolor photographic elements contain a dye image forming compound. The dye image can be formed by the selective destruction, formation or physical removal of dyes. Element constructions that form images by the physical removal of preformed dyes are illustrated by *Research Disclosure*, Vol. 308, December 1989, Item 308119, Section VII. Color materials, paragraph H. Element constructions that form images by the destruction of dyes or dye precursors are illustrated by *Research Disclosure*, Item 36544, previously cited, Section X. Dye image formers and modifiers, Subsection A. Silver dye bleach. Dye-forming couplers are illustrated by *Research Disclosure*, Item 36544, previously cited, Section X. Subsection B. Image-dye-forming couplers. It is also contemplated to incorporate in the emulsion layer units dye image modifiers, dye hue modifiers and image dye stabilizers, illustrated by *Research Disclosure*, Item 36544, previously cited, Section X. Subsection C. Image dye modifiers and Subsection D. Hue modifiers/stabilization. The dyes, dye precursors, the above-noted related addenda and solvents (e.g., coupler solvents) can be incorporated in the emulsion layers as dispersions, as illustrated by *Research Disclosure*, Item 36544, previously cited, Section X. Subsection E. Dispersing and dyes and dye precursors.

20 Materials useful in the preparation of color papers are further illustrated by current commercial practice as, for example, by EDGE™, PORTRA™ or SUPRA™, Color Papers as sold by Eastman Kodak Company, by FUJI™ FA-family Color Papers and FUJI Type D Digital Paper as sold by Fuji Photo Film, by KONICA™ QA-family Color Papers as sold by Konishiroku Industries, by DURATRANS™ and DURACLEAR™ display films as sold by Eastman Kodak Company and by KONSENSUS-II™ display films as sold by Konishiroku Industries. It is also contemplated that the emulsion composition of the invention may be advantageously incorporated into the 25 elements described in an article titled "Typical and Preferred Color Paper, Color Negative, and Color Reversal Photographic Elements and Processing," published in *Research Disclosure*, February 1995, Item 37038. The advantages of the current invention may be achieved by modifying any of 30 these formulations to conform to the requirements set forth in the specification. The exact magnitude of the benefits achieved will, of course, depend on the exact details of the 35 formulations involved but these will be readily apparent to the skilled practitioner.

40 45 50 55 60 65 Silver halide emulsions satisfying the grain requirements described above can be present in any one or combination of the emulsion layer units. Additional useful multicolor, multilayer formats for an element of the invention include Structures I-IV as described in U.S. Pat. No. 5,783,373 referenced above, which is incorporated by reference herein. Each of such structures in accordance with the invention would contain at least one silver halide emulsion comprised

of high chloride grains as described above. In accordance with preferred embodiments, at least the blue-sensitized, yellow dye image-forming unit of such elements comprises such a high chloride emulsion. Preferably each of the emulsion layer units contain an emulsion satisfying these criteria.

Conventional features that can be incorporated into multilayer (and particularly multicolor) recording elements contemplated for use in the method of the invention are also illustrated by *Research Disclosure*, Item 38957, cited above:

- XI. Layers and layer arrangements
- XII. Features applicable only to color negative
- XIII. Features applicable only to color positive
- B. Color reversal
- C. Color positives derived from color negatives

XIV. Scan facilitating features.

The recording elements comprising the radiation sensitive iodide-banded high chloride emulsion layers according to this invention can be image-wise exposed in a pixel-by-pixel mode using suitable high energy radiation sources typically employed in electronic printing methods. In one further embodiment, the present invention is accordingly directed to an electronic printing method which comprises subjecting a radiation sensitive silver halide emulsion layer of a recording element to actinic radiation of at least  $10^{-4}$  ergs/cm<sup>2</sup> for up to  $100\mu$  seconds duration in a pixel-by-pixel mode. The present invention realizes an improvement in reciprocity failure by modifying the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

Suitable actinic forms of energy for exposing light sensitive recording elements in accordance with the invention encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appropriate spectral radiation, for example, infrared, red, green or blue wavelengths, to which such element is sensitive. Multicolor elements can be employed which produce cyan, magenta and yellow dyes as a function of exposure in separate portions of the electromagnetic spectrum, including at least two portions of the infrared region, as disclosed in the previously mentioned U.S. Pat. No. No. 4,619,892, incorporated herein by reference. Suitable exposures include those up to 2000 nm, preferably up to 1500 nm. The exposing source need, of course, provide radiation in only one spectral region if the recording element is a monochrome element sensitive to only that region (color) of the electromagnetic spectrum. Suitable light emitting diodes and commercially available laser sources are described in the examples. Imagewise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

The quantity or level of high energy actinic radiation provided to the recording medium by the exposure source is

generally at least  $10^{-4}$  ergs/cm<sup>2</sup>, typically in the range of about  $10^{-4}$  ergs/cm<sup>2</sup> to  $10^{-3}$  ergs/cm<sup>2</sup> and often from  $10^{-3}$  ergs/cm<sup>2</sup> to  $10^{-2}$  ergs/cm<sup>2</sup>. Exposure of the recording element in a pixel-by-pixel mode as known in the prior art persists for only a very short duration or time. Typical maximum exposure times are up to  $100\mu$  seconds, often up to  $10\mu$  seconds, and frequently up to only  $0.5\mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988, which is hereby incorporated herein by reference. A description of some of the details of conventional electronic printing methods comprising scanning a recording element with high energy beams such as light emitting diodes or laser beams, are set forth in Hioki U.S. Pat. No. 5,126,235, European Patent Applications 479 167 A1 and 502 508 A1, the disclosures of which are hereby incorporated herein by reference.

Once imagewise exposed, the recording elements can be processed in any convenient conventional manner to obtain a viewable image. Such processing is illustrated by *Research Disclosure*, Item 38957, cited above:

XVIII. Chemical development systems

XIX. Development

XX. Desilvering, washing, rinsing and stabilizing

The described elements can be also processed in the ionic separation imaging systems which utilize the sulfonamidonaphthol diffusion transfer technology. Such a photographic product comprises at least one image dye providing element comprising at least one layer of photosensitive silver halide emulsion with which is associated a non-diffusible image dye-providing substance. After image-wise exposure, a coating is treated with an alkaline processing composition in the presence of a silver halide developing agent in such a way that for each dye-image forming element, a silver image is developed. An image-wise distribution of oxidized developer cross-oxidizes the molecule of the image dye-providing compound. This, in an alkaline medium, cleaves to liberate a diffusible image dye. A preferred system of this type is disclosed in Fleckenstein U.S. trial voluntary protest document B351,637, dated Jan. 28, 1975. Other patents include: U.S. Pat. Nos. 4,450,224 and 4,463,080, and U.K. Patents 2,026,710 and 2,038,041.

In a similar technology, a silver halide photographic process is combined with LED exposure and thermal development/transfer resulting in a high image quality hard copy system incorporating digital exposure technology. Some of the many patents include U.S. Pat. Nos. 4,904,573; 4,952,969; 4,732,846; 4,775,613; 4,439,513; 4,473,631; 4,603,103; 4,500,626; 4,713,319.

The following examples illustrate the practice of this invention. They are not intended to be exhaustive of all possible variations of the invention. Parts and percentages are by weight unless otherwise specified.

EXAMPLES

Example 1

To a reactor incorporating a stirring device as disclosed in *Research Disclosure*, Item 38213, and containing 8.84 kg of

19

distilled water, 25 mg of p-glutaramidophenyl disulfide and 250 g of bone gelatin, were added 291 g of 3.8 M sodium chloride salt solution such that the mixture was maintained at a pCl of about 1.05 at approximately 68° C. To this were added 1.9 of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a constant silver nitrate flow rate of about 240 mL/min for about 1 minute while maintaining pCl constant at about 1.05. Following this nucleation period the rest of silver nitrate and sodium chloride for growth of the 92% of the core grain were delivered with five pulses at the flow rate of about 232 mL/min separated by hold periods. Then both the silver and sodium salt solution pumps were turned off and about 1.6 M potassium iodide solution was added to the stirred reaction mixture over about 30 seconds at a constant flow rate of about 62.9 mL/min. The resultant iodochloride emulsion was then grown further by pulsed controlled double-jet addition for about 1.26 minutes by resumed addition of silver and sodium salt solutions at about 223 mL/min at a pCl of about 1.05. In addition, cesium pentachloronitrosylsulfate was added at approximately 4 to 70% into the precipitation, potassium hexacyanoruthenate at 76-81%, and iridium pentachloro-5-methylthiazole at 93-95% band after iodide addition. A silver iodochloride emulsion was thus prepared with 0.4 mole % iodide located at 92% of total grain volume. Cubic edge length was 0.51  $\mu$ m.

A portion of this silver chloroiodide emulsion was optimally sensitized by adjusting the pH to 5.6 with 10% nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of Lippmann bromide (in the amount of 0.17 mole % based on total silver) and 107 mg/Ag mole of 1-(3-acetamidophenyl)-5-mercaptopotetrazole.

Dye 1



## Example 2

To a reactor incorporating a stirring device as disclosed in *Research Disclosure*, Item 38213, and containing 8.84 kg of distilled water, 25 mg of p-glutaramidophenyl disulfide and 250 g of bone gelatin, were added 291 g of 3.8 M sodium chloride salt solution such that the mixture was maintained at a pCl of about 1.05 at approximately 68° C. To this were added 1.9 of 1,8-dihydroxy-3,6-dithiaoctane approximately 30 seconds before commencing introduction of silver and chloride salt solutions. Aqueous solutions of about 3.7 M silver nitrate and about 3.8 M sodium chloride were then added by conventional controlled double-jet addition at a

20

constant silver nitrate flow rate of about 240 mL/min for about 1 minute while maintaining pCl constant at about 1.05. Following this nucleation period the rest of silver nitrate and sodium chloride for growth of the 92% of the core grain were delivered with five pulses at the flow rate of about 232 mL/min separated by hold periods. Then both the silver and sodium salt solution pumps were turned off and silver iodide Lippmann emulsion was added to the reactor in the amount equivalent to 0.4 mole percent of the total halide content of the final emulsion. The resultant iodochloride emulsion was then grown further by pulsed controlled double-jet addition for about 1.26 minutes by resumed addition of silver and sodium salt solutions at about 223 mL/min at a pCl of about 1.05. In addition, cesium pentachloronitrosylsulfate was added at approximately 4 to 70% into the precipitation, potassium hexacyanoruthenate at 76-81%, and iridium pentachloro-5-methylthiazole at 93-95% band after iodide addition. A silver iodochloride emulsion was thus prepared with 0.4 mole % iodide located at 92% of total grain volume. Cubic edge length was 0.51  $\mu$ m.

A portion of this silver chloroiodide emulsion was optimally sensitized by adjusting the pH to 5.6 with 10% nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of Lippmann bromide (in the amount of 0.17 mole % based on total silver) and 107 mg/Ag mole of 1-(3-acetamidophenyl)-5-mercaptopotetrazole.

## Example 3

Emulsion in this example was precipitated as in Example 2, with the following exception: total amount of iodide was 0.6 mole percent of the total halide content.

A portion of this silver chloroiodide emulsion was optimally sensitized by adjusting the pH to 5.6 with 10% nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of Lippmann bromide (in the amount of 0.17 mole % based on total silver) and 107 mg/Ag mole of 1-(3-acetamidophenyl)-5-mercaptopotetrazole.

## Example 4

A portion of the emulsion precipitated in Example 1 was optimally sensitized by adjusting the pH to 5.6 with 10% nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of 0.022 mg/Ag mole of potassium hexachloroiridate and Lippmann bromide (in the amount of 0.17 mole % based on total silver). Finally 107 mg/Ag mole of 1-(3-acetamidophenyl)-5-mercaptopotetrazole was added.

## Example 5

A portion of the emulsion precipitated in Example 2 was optimally sensitized by adjusting the pH to 5.6 with 10%

nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of 0.022 mg/Ag mole of potassium hexachloroiridate and Lippmann bromide (in the amount of 0.17 mole % based on total silver). Finally 107 mg/Ag mole of 1-(3-acetamidophenyl)-5-mercaptop tetrazole was added.

## Example 6

A portion of the emulsion precipitated in Example 3 was optimally sensitized by adjusting the pH to 5.6 with 10% nitric acid solutions and adjusting the pAg to 7.6 with sodium chloride solution, both at 40° C., followed by the addition of 10 mg/Ag mole of p-glutaramidophenyl disulfide and 20.4 mg/Ag mole of a colloidal suspension of aurous sulfide. The emulsion was then heated up to 60° C. and 450 mg/Ag mole of blue sensitizing dye—Dye1 was added followed by the addition of 0.022 mg/Ag mole of potassium hexachloroiridate and Lippmann bromide (in the amount of 0.17 mole % based on total silver). Finally 107 mg/Ag mole of 1-(3-acetamidophenyl)-5-mercaptop tetrazole was added.

Blue sensitized emulsions from Example 1, 2, 3, 4, 5, and 6 were coated at 19.5 mg silver per square foot and coupler dispersion Y-1 at 50 mg per square foot. The coatings were overcoated with gelatin layer and the entire coating was hardened with bis(vinylsulfonylmethyl)ether.



Single layer samples were exposed for 0.1 second to simulate exposure through a color negative film. 0-3.0 density step tablet was used and the source of white light was a Kodak Model 1B sensitometer with a color temperature of 3000° K and with a combination of the appropriate filters. The samples were also exposed through a step wedge with 3000° K tungsten source at high-intensity short exposure times ( $10^{-5}$  second) or low-intensity long exposure time of  $10^{-2}$  second. The total energy of each exposure was kept at a constant level. Further, the samples were exposed with blue laser exposing device using Argon Ion (multiline) laser at 467.5 nm at a resolution of 196.8 pixels/cm and a pixel pitch of 50.8  $\mu$ m, and the exposure time of 1 microsecond per pixel. The exposed coatings were processed using Kodak™ Ektacolor RA-4 processing.

Long-time flash exposure Relative log speed was measured at 0.8 absolute density at  $1/10^{th}$  second exposure time.

Short-time flash exposure Relative log speed was measured at 2.0 absolute density at  $10^{-5}$  second exposure time.

Short time Ar<sup>+</sup> laser exposure Relative log speed was measured at 2.0 absolute density at pixel time 1 microsecond at the wavelength of 467.5 nm.

High Intensity Reciprocity Failure (HIRF) is reported as the speed difference between equal energy exposures at  $10^{-5}$

and  $10^{-2}$  second exposure time, measured at an absolute density equal 2.0.

TABLE 1

| Composite iodobromochloride grains with iridium added during chemical sensitization. |                           |                                                  |                                               |                                                |                                                |      |  |
|--------------------------------------------------------------------------------------|---------------------------|--------------------------------------------------|-----------------------------------------------|------------------------------------------------|------------------------------------------------|------|--|
| Example                                                                              | KI/AgI level/<br>location | Iridium<br>added at<br>chem-<br>ical<br>ripening | Long-time<br>flash<br>exposure:<br>Rel. speed | Short-time<br>flash<br>exposure:<br>Rel. speed | Short-time<br>laser<br>exposure:<br>Rel. speed | HIRF |  |
| 1 Comparison                                                                         | KI at 0.4/92%             | no                                               | 100.0                                         | 100.0                                          | 100.0                                          | -34  |  |
| 2 Comparison                                                                         | AgI at 0.4/92%            | no                                               | 94.6                                          | 106.0                                          | 110.1                                          | -29  |  |
| 3 Comparison                                                                         | AgI at 0.6/92%            | no                                               | 109.5                                         | 119.0                                          | 114.5                                          | -28  |  |
| 4 Comparison                                                                         | KI at 0.4/92%             | yes                                              | 103.3                                         | 106.0                                          | 106.4                                          | -29  |  |
| 5                                                                                    | AgI at 0.4/92%            | yes                                              | 85.6                                          | 137.0                                          | 124.3                                          | +2   |  |
| Invention                                                                            | 0.4/92%                   |                                                  |                                               |                                                |                                                |      |  |
| 6                                                                                    | AgI at 0.6/92%            | yes                                              | 97.6                                          | 143.0                                          | 128.0                                          | +2   |  |
| Invention                                                                            | 0.6/92%                   |                                                  |                                               |                                                |                                                |      |  |

## Example 7

Emulsion in this example was prepared in an identical manner as in Example 1.

## Example 8

Emulsion in this example was prepared in an identical manner as in Example 2.

## Example 9

Emulsion in this example was prepared in an identical manner as in Example 4.

## Example 10

Emulsion in this example was prepared in an identical manner as in Example 5.

Blue sensitized emulsions from Example 7 through Example 10 were coated as “Yellow emulsion YE1” in the following multialyer format:

| Format 1 |                             |                            |
|----------|-----------------------------|----------------------------|
|          | Item Description            | Lavdown mg/ft <sup>2</sup> |
| Layer 1  | Blue Sensitive Layer - 1    |                            |
|          | Gelatin                     | 140                        |
|          | Yellow emulsion YE1 (as Ag) | 26                         |
|          | Y-2                         | 60                         |
|          | ST-1                        | 13.75                      |
|          | S-2                         | 26.25                      |
| Layer 2  | Interlayer - 1              |                            |
|          | Gelatin                     | 30                         |
|          | Y-2                         | 18                         |
|          | ST-1                        | 4.1                        |
|          | S-2                         | 7.9                        |
| Layer 3  | Interlayer 2                |                            |
|          | Gelatin                     | 70                         |
|          | SC-1                        | 6                          |
|          | S-1                         | 17.9                       |
| Layer 4  | Green Sensitive Layer       |                            |
|          | Gelatin                     | 124.5                      |
|          | Magenta emulsion (as Ag)    | 9.7                        |
|          | M-1                         | 20.9                       |

-continued

| Format 1             |                            |
|----------------------|----------------------------|
| Item Description     | Lavdown mg/ft <sup>2</sup> |
| S-2                  | 7.4                        |
| ST-2                 | 5.6                        |
| ST-3                 | 15.9                       |
| ST-4                 | 53                         |
| PMT                  | .025                       |
| Layer 5              | UV Interlayer              |
| Gelatin              | 66.1                       |
| UV-1                 | 2.8                        |
| UV-2                 | 16                         |
| SC-1                 | 5.13                       |
| S-1                  | 3                          |
| S-3                  | 3                          |
| Layer 6              | Red Sensitive Layer        |
| Gelatin              | 124.3                      |
| Cyan emulsion CE1    | 19.6                       |
| C-1                  | 39.4                       |
| S-1                  | 34.7                       |
| UV-2                 | 22.8                       |
| S-4                  | 2.9                        |
| SC-1                 | 0.3                        |
| Layer 7              | UV Overcoat                |
| Gelatin              | 49.9                       |
| UV-1                 | 1.2                        |
| UV-2                 | 6.9                        |
| SC-1                 | 2.2                        |
| S-1                  | 1.2                        |
| S-3                  | 1.2                        |
| Layer 8              | SOC                        |
| Gelatin              | 60                         |
| Polydimethylsiloxane | 1.88                       |
| Ludox Am™            | 15                         |



S-1 = dibutyl phthalate

-continued

| Format 1         |                            |
|------------------|----------------------------|
| Item Description | Lavdown mg/ft <sup>2</sup> |
| SC-1             |                            |
| 10               |                            |
| 15               |                            |
| 20               |                            |
| 25               |                            |
| 30               |                            |
| 35               |                            |

PMT = 1-phenyl-5-mercaptopentetrazole



UV-1



55 Each of the multicolor, multilayer coatings was exposed by a 1700 Lux tungsten lamp with a 3000° K temperature for 0.5 seconds. Filtration for the red sensitive layer was a Wratten 70, for the green sensitive layer a Wratten 99+0.3 neutral density, and for the blue Wratten 48+2B+0.8 neutral density. Further, the samples were exposed with blue laser exposing device using Argon Ion (multiline) laser at 467.5 nm at a resolution of 196.8 pixels/cm and a pixel pitch of 50.8  $\mu$ m, and the exposure time of 1 microsecond per pixel. The exposed samples were processed in Kodak™ Ektacolor RA-4 processing chemistry in a roller transport processor. Emulsion coating performance was judged by measuring (a) photographic speed for the Long-time flash (0.5 seconds)

exposure in relative Log exposure units at a density of 0.8, (b) an upper scale laser speed for the Short-time laser exposure (measured at density=2.0), (c) emulsion contrast measured as a "shoulder" density on the laser-generated D-Log E curve that is one unit of log E removed from the point defined by minimum density plus 0.04 (this is a very important measure of the "dynamic range" offered by an emulsion in digital exposing devices).

TABLE 2

Composite iodobromochloride grains with iridium added during chemical sensitization and coated in color paper multilayer

| Example       | KI/AgI level/ location | Iridium added at chemical ripening | Long-time flash exposure: Rel. speed | Short-time laser exposure: Rel. speed | Contrast (Dynamic Range) |
|---------------|------------------------|------------------------------------|--------------------------------------|---------------------------------------|--------------------------|
| 7             | KI at 0.4/92%          | no                                 | 100.0                                | 100.0                                 | 1.350                    |
| Comparison 8  | AgI at 0.4/92%         | no                                 | 93.7                                 | 109.0                                 | 1.604                    |
| Comparison 9  | KI at 0.4/92%          | yes                                | 104.8                                | 108.0                                 | 1.506                    |
| Comparison 10 | AgI at 0.4/92%         | yes                                | 85.6                                 | 128.0                                 | 1.894                    |
| Invention     | 0.4/92%                |                                    |                                      |                                       |                          |

It is specifically contemplated that emulsions in accordance with the invention may be sensitized with red, green, and blue sensitizing dyes and be incorporated in a color paper format as described in Example 4 of U.S. Pat. No. 5,783,373, incorporated by reference above. It is also specifically contemplated to employ emulsions in accordance with the invention in place of the Yellow emulsion YE1 in "Format 1" of the Examples of concurrently filed, copending, commonly assigned U.S. Ser. No. 09/475,405 (Kodak Docket 80210A1A) incorporated by reference above.

The invention has been described in detail with particular reference to preferred embodiments thereof, but it will be understood that variations and modifications can be effected within the spirit and scope of the invention.

What is claimed is:

1. A process for the preparation of a radiation-sensitive silver halide emulsion comprised of high chloride cubical host grains containing from 0.05 to 3 mole percent iodide, based on total silver, and epitaxially deposited silver bromide, where the iodide is incorporated in the host grains in a controlled, non-uniform distribution forming a core containing at least 50 percent of total silver, an iodide free surface shell having a thickness of greater than 50 Å, and a sub-surface shell that contains a maximum iodide concentration, the process comprising:

- providing in a stirred reaction vessel a dispersing medium and high chloride silver halide cubical grains which form the high chloride host grain cores,
- adding fine silver iodide grains to the reaction vessel and ripening out the fine silver iodide grains to form the sub-surface shells that contain a maximum iodide concentration,
- precipitating silver chloride onto the sub-surface shells to form an iodide free surface shell, and
- depositing silver bromide in an amount of from 0.05 to 5 mole percent, based on total silver, on the host grain surfaces in the presence of an iridium dopant.

2. A process according to claim 1, wherein the iridium dopant is a coordination complex of the formula:



wherein

n is zero, -1, -2, -3 or -4; and

$\text{L}_6$  represents six bridging ligands which can be independently selected, provided that at least four of the ligands are anionic ligands.

3. A process according to claim 2 wherein at least one of the ligands of the dopant is a halide ligand.

4. A process according to claim 2 wherein at least four of the ligands of the dopant are halide ligands.

5. A process according to claim 2 wherein at least one of the ligands of the dopant is a chloride ligand.

6. A process according to claim 2 wherein at least four of the ligands of the dopant are chloride ligands.

7. A process according to claim 2 wherein the dopant comprises an iridium hexahalo coordination complex.

8. A process according to claim 7 wherein the dopant comprises an iridium hexachloro coordination complex.

9. A process according to claim 8, wherein silver bromide is deposited on the host grain surfaces in the presence of an iridium dopant in step (d) in an amount of from 0.1 to 1 mole percent, based on total silver.

10. A process according to claim 9 wherein the iridium dopant is present during step (d) at a concentration of from 0.0001 to 1.0 mg/silver mole.

11. A process according to claim 9 wherein the iridium dopant is present during step (d) at a concentration of from 0.001 to 0.1 mg/silver mole.

12. A process according to claim 1, wherein the high chloride cubical host grains contain from 0.1 to 1 mole percent iodide, based on total silver.

13. A process according to claim 1 wherein the silver halide grains contain at least 70 mole percent chloride, based on silver.

14. A process according to claim 1 wherein the silver halide grains contain at least 90 mole percent chloride, based on silver.

15. A photographic element comprising a support having coated thereon a radiation sensitive emulsion layer comprising a high chloride emulsion according to claim 1.

16. A photographic element according to claim 15, comprising a blue-light sensitive emulsion layer comprising a high chloride emulsion according to claim 1.

17. An electronic printing method comprising subjecting a radiation sensitive silver halide emulsion layer of a photographic element according to claim 15 to actinic radiation of at least  $10^{-4}$  ergs/cm<sup>2</sup> for up to 100 $\mu$  seconds duration in a pixel-by-pixel mode.

18. A method according to claim 17 wherein the exposure is up to 10 microseconds.

19. A method according to claim 17 wherein the duration of the exposure is up to 0.5 microseconds.

20. A method according to claim 17 wherein the duration of the exposure is up to 0.05 microseconds.

21. A method according to claim 17 wherein the source of actinic radiation is a light emitting diode.

22. A method according to claim 17 wherein the source of actinic radiation is a laser.

23. A method according to claim 17 wherein the pixels are exposed to actinic radiation of about  $10^{-3}$  ergs/cm<sup>2</sup> to  $10^2$  ergs/cm<sup>2</sup>.